

## UNITED STATES PATENT OFFICE

2,164,237

## TREATING TEXTILES AND OILS THEREFOR

Walter Garner, Menston-in-Wharfedale,  
EnglandNo Drawing. Application July 16, 1937, Serial  
No. 154,072. In Great Britain January 21,  
1936

3 Claims. (Cl. 19—66)

This invention relates to improvements in treating textile materials consisting of or containing animal hairs such as wool, mohair, angora, recovered wool (e. g., shoddy) either alone or mixed with each other or with other fibres, e. g., silk, rayon or cotton.

This invention relates also to improvements in treating textile materials other than animal hairs, such as silk, rayon, cotton and caseine wool, either alone or mixed with each other or with other fibres.

In dealing with such materials it is frequently necessary to treat them with a lubricant which must subsequently be removable by ordinary scouring operations. Olive oil is generally used for this purpose but many other substances have been proposed. It is difficult, however, to find a substitute for olive oil which is reasonably cheap and satisfies the requirements of a textile lubricant, especially the somewhat exacting requirements of the worsted industry.

The invention is particularly applicable in the worsted industry in which a high grade oil is used and removed by scouring with soap as distinct from the woollen industry in which large quantities of cheaper acid oils are used and usually scoured with alkali.

According to the invention such textile materials either in the loose form, or as sliver, yarn or fabric or in intermediate stages of processing or in other form, are treated with an ester or mixture of esters as hereinafter defined, and after subjecting the treated materials to one or more textile operations (e. g., carding, combing, spinning, weaving or knitting), they are then scoured.

The esters according to the invention are synthetic esters of alcohols having less than 3 hydroxy groups and in which the carboxyl groups are fully esterified; these synthetic esters are chosen so as to be comparatively resistant to oxidation and substantially insoluble in water but capable of being emulsified by the liquids employed in the scouring operation, and are such polymerised and/or oxidised esters as have these properties. By polymerised and/or oxidised esters are meant esters formed either by combining an alcohol having less than 3 hydroxy groups with an unsaturated fatty acid which has been polymerised and/or oxidised or by forming an ester of an alcohol having less than 3 hydroxy groups and unsaturated acid and polymerising and/or oxidising such ester. The esters defined above are oily bodies; they are therefore distinguished from esters which are capable of

dissolving or dispersing in water alone and which have wetting and foaming powers enabling them to be used as substitutes for soaps and Turkey red oils.

In defining the above oily bodies as resistant to oxidation, we mean that they should not oxidise much more easily than olive oil of the quality usually used for textile purposes when tested by standard available tests. Moreover, although insoluble in water and not capable of dispersing therein alone by simple agitation, they must be sufficiently readily emulsifiable in the scouring bath employed, e. g., soap solution with or without alkali, to be removed, practically speaking, in the scouring operation. They should compare favourably with olive oil in both these respects.

Preferably both the alcohol and acid are of high molecular weight and in any case the fatty acid contains more than eight carbon atoms.

The most suitable alcohols which must have less than three hydroxy groups have six or more carbon atoms. Examples are hexyl alcohol, lauryl alcohol, cetyl alcohol, cholesterol, methyl cyclohexanol, ethylene glycol, propylene glycol, or the simple substitution products of such alcohols, though ethyl alcohol may be used also.

The most suitable acids are monoethenoid fatty acids (e. g., oleic acid) and their simple substitution products (e. g., ricinoleic acid). Although the esters of such acids are usually of the same order of stability as the triglyceride of oleic acid to oxidation by exposure to air, they respond to polymerisation or oxidation by virtue of the presence of an ethenoid linkage.

Less suitable acids are the diethenoid fatty acids, e. g., linoleic acid, and their simple substitution products. Although the esters of such acids are more easily oxidised than the triglyceride of oleic acid by exposure to air they can be employed either alone or in admixture with monoethenoid fatty acids to produce products which may be inferior so far as resistance to oxidation is concerned, to those products prepared only from monoethenoid fatty acids, but superior in certain other respects, e. g., cost.

Unsaturated acids of the types mentioned above which have been oxidised or hydrogenated, and simple substitution products of such modified acids, may also be employed.

Acids of any of the types mentioned above may be used either alone or in admixture with each other or in admixture with saturated fatty acids which act as diluents, e. g., stearic acid.

Synthetic esters formed by combination of suitable alcohols and fatty acids, which have after

formation been partially hydrogenated, or simple substitution products of such partially hydrogenated esters, may also be polymerised and/or oxidised to yield textile oils according to the invention.

The compositions employed for treating the textile materials may consist of the pure or commercial esters as defined above or mixtures thereof with a diluent such as mineral oil or a solid ester or with a substance which assists emulsification, or aqueous emulsions may be used. Substances of a higher or lower viscosity may be added respectively to increase or reduce the viscosity. Thus castor oil or polymerised rape oil may be added to increase the viscosity or a thin mineral oil or thin ester may be added to reduce the viscosity.

It has already been stated that the ester must be readily emulsifiable. It must emulsify fairly easily with soap solution with or without alkali. The diluent need not necessarily comply with this condition provided the mixture does so. The behaviour when present upon wool fibre is ascertained for example by the following scouring test:

25 A wool hank is steeped in a 3½% solution of the oil in a volatile organic solvent, squeezed, and allowed to stand 12 hours to ensure a complete and even impregnation. The hank is then secured in a solution of 0.2% soap and 0.1% ammonia at 45° C. for one quarter of an hour in an apparatus which circulates the liquor. It is then washed in water, dried, and the percentage residual oil is ascertained. This test corresponds to a trade method of scouring wool hanks.

35 The textile oil composed entirely or partly of an ester according to the invention should have a viscosity between 200 and 650 seconds Redwood at 60° F. The preferred compositions have a viscosity between 300 and 500 seconds Redwood 40 at room temperature and a flash point above 330° F., as these qualities enable them to satisfy current requirements in the trade although they are not essential for practical success.

By way of example oxidised and slightly polymerised methyl cyclohexanol oleate may be prepared from commercial methyl cyclohexanol by esterification with oleic acid and subsequent oxidation and slight polymerisation by blowing the heated ester with air or even by agitation in presence of air. Such a product, having for example an iodine value of 51, may be used as a substitute for olive oil (iodine value 88). This product is so little sensitive to oxidation as compared to ordinary textile olive oil that after two hours in the Mackey testing apparatus the temperature was only 215° F. (olive oil 490° F.).

Two parts of this oxidised and slightly polymerised methyl cyclohexanol oleate may be emulsified by the aid of one part of soap solution to form a "wool cream" which is suitably diluted before use. Twitchell base may also be used as the emulsifier.

By working according to this invention it is possible to produce oils which are even superior to olive oil in one or more of the following properties: absence of rancidity, reduced colour, and reduced odour.

I claim as my invention:

1. Process of treating textile materials which consists in oiling the material with an oxidised ester containing a cyclohexanol nucleus and a fatty acid radical containing more than eight carbon atoms having a viscosity between 200 and 650 seconds Redwood at 60° F., and being comparatively resistant to oxidation, and substantially insoluble in water but capable of being emulsified by a scouring liquid, subjecting the oiled material to at least one mechanical textile process, and scouring the material.
2. Process as in claim 1, in which a diluent is used with the synthetic ester.
3. Process as in claim 1 in which the synthetic ester is used in the form of an emulsion.

WALTER GARNER.